

Aug. 27, 1929.

F. K. HABENICHT ET AL

1,726,180

FORGED JOURNAL BEARING WEDGE AND PROCESS OF MAKING SAME

Filed May 25, 1928

Fig. 1.



Fig. 2.



Fig. 3.



Inventors

F. K. Habenicht  
F. H. Pietzsch

By *E. C. Kupferman*  
Att'y.

## UNITED STATES PATENT OFFICE.

FREDERICK K. HABENICHT AND FRANK H. PIETZSCH, OF ST. LOUIS, MISSOURI, ASSIGNEES TO RAILWAY DEVICES COMPANY, OF ST. LOUIS, MISSOURI, A CORPORATION OF MISSOURI.

## FORGED JOURNAL-BEARING WEDGE AND PROCESS OF MAKING SAME.

Application filed May 25, 1928. Serial No. 280,514.

It is desirable that wedges for railway journal bearings have flat side bearings extending substantially from the top to the bottom of the wedge to effectively prevent 5 the tilting of the wedge under torsional strain imparted from the axle to the brass and its cooperating wedge particularly when the car is started or stopped. Such 10 extended flat side bearings may be readily produced on cast wedges but in drop forged wedges, as heretofore produced, only a flat flash line of about one quarter inch in width is produced, the remainder of the side bearing tapering toward the top and bottom of 15 the wedge in order to provide the necessary draft to prevent the wedge from adhering to the forging dies. It is of course possible to provide such drop forged wedges with extended side bearings by machining or grind- 20 ing operations but this so increases the cost that they cannot be sold in competition with cast wedges.

It is the object of our invention to produce a drop forged wedge with extended 25 flat side bearings without resorting to supplementary machining or grinding operations.

In the accompanying drawings, which illustrate a wedge made in accordance with 30 our invention, Figure 1 is a perspective view of the wedge before the flash is trimmed; Figure 2 is a perspective view of the completed wedge; and Figure 3 is a view illustrating the manner of forming the flat side 35 bearings by trimming.

The wedge 5 as shown in the drawings is in general conformation of the usual M. C. B. type and is interchangeable therewith. It is drop forged, a flash 6 being formed at 40 the meeting line of the forging dies. Each of the side bearings consists of an upper

part 7 and a pair of lower parts 8 out of vertical alignment with the upper part. These parts 7 and 8 are so proportioned as to project slightly beyond the contour of 45 the finished wedge. At the same time that the flash 6 is trimmed to produce the flash line 6' the parts 7 and 8 are also trimmed, as shown in dotted lines in Figure 3, so that a flat side bearing 7', 8' is produced 50 extending from the top to the bottom of the wedge. The result we are enabled to accomplish by reason of the offset arrangement of the parts 7 and 8, for we have found that while the entire thickness of the 55 metal of the wedge offers more resistance than can be overcome by the trimming die, one-half the thickness can be successfully severed and with the offset arrangement of the parts 7 and 8 this is all the metal under 60 shearing strain at any one time during the operation of trimming.

It will be seen that by our method we produce a forged wedge having flat side bearings extending from the top to the bottom of the 65 wedge without any increase in cost of production over the ordinary drop forged wedges having inclined side bearings.

Having fully described our invention, what we claim as new and desire to secure 70 by Letters Patent of the United States is:

The method of forming journal bearing wedges which comprises forging the wedge with a flash and with a side projection, and simultaneously trimming said flash and projection to form a flat side bearing extending in a vertical direction from the flash line.

In testimony whereof, we hereunto affix our signatures, this 23rd day of May, 1928.

FREDERICK K. HABENICHT.  
FRANK H. PIETZSCH.